

# UNITED STATES PATENT OFFICE.

FREDUS ALEXANDER THURSTON, OF CHICAGO, ILLINOIS.

## METHOD OF MAKING GOLD INLAYS.

1,209,906.

Specification of Letters Patent. Patented Dec. 26, 1916.

No Drawing.

Application filed July 26, 1911. Serial No. 640,595.

To all whom it may concern:

Be it known that I, FREDUS A. THURSTON, a citizen of the United States, residing at Chicago, in the county of Cook and State of Illinois, have invented a certain new and useful Improvement in Methods of Making Gold Inlays, of which the following is a full, clear, concise, and exact description.

The object of this invention is to provide 10 a method of making metal objects for dental or other work which shall be accurate and at the same time rapid and economical.

A further object is to avoid the use of 15 special apparatus in making inlays of gold or other metal. The method described herein while developed primarily for use with gold has been applied successfully in making platinum and silver inlays. An essential and 20 the first step in the process is the preparation of a metal sponge of a high melting point. This sponge may be prepared in any quantity desired and kept in readiness for dental or other operations.

In preparing the gold sponge, moss fiber 25 gold or any preparation equally as spongy may be used. The spongy gold is mixed with a binder, which binder may be prepared as follows: Mix a small quantity of cocoanut oil with resin, sufficient to make 30 a gum that will not quite run when cool. This is done by heating the resin and adding the oil in sufficient quantity. The gum is then added to the gold by dipping therein a flat instrument and carrying threads 35 of the stringy gum over the mat of sponge gold sufficiently close together so that when melted the entire surface of the resulting mixture will be pretty well permeated with gum. The tendency is to get too much gum 40 in the gold. The resulting gold mat is then placed on a surface which can be evenly heated and brought to a temperature where the gum will smoke, whereupon the heating is stopped. Care should be taken to 45 prevent the gold in any part becoming red hot as that will make it granular. The resulting sponge is slightly sticky even in the presence of moisture and retains a considerable degree of porosity, so that after polishing, the pores of the sponge are not completely closed.

While the preceding method of preparing the binder and sponge is the preferred method it will be obvious to those who have

had experience with gums and oils that a 55 number of substances may be substituted for the resin, such as beeswax, paraffin, shellac or other equivalents. Moreover, other oils than cocoanut oil may be used such as light cotton seed oil or any oil which is capable 60 of dissolving the gummy material used. In fact the particular binder used is not an essential feature of my invention, but any binding material may be used which will retain its porosity and which can be eliminated 65 without destroying the form of the sponge. It has been found also that borax may be used with the resin or other gum. While this method was originally developed in connection with gold sponge, it has been found 70 that the method may be applied to substances which are not metallic in their nature, such as silica, it only being necessary that the material used as a base for the original sponge shall be somewhat refractory so that the binder may be driven off and the filling material fused into place without 75 destroying the form of the article desired. It will be seen also that wherever in the specification metal is referred to as being 80 fused into the sponge, other material might be used as a filler instead of metal, the only requirement being that the fused material used for filling the pores of the sponge shall have a lower melting point than the material used as the base in forming the sponge. 85

In using the prepared sponge for making gold inlays in case of simple cavities with walls sufficiently sloped outward a matrix may not be necessary, but the inlay may be 90 prepared as follows: Oil the cavity and select a piece of treated sponge gold in bulk several times larger than the space to be filled and with a burnisher force the cavity full and compact, leaving the cavity slightly 95 overfull. If more sponge is used than necessary it may be trimmed away with a warm instrument, while if more is required it may be applied since the sponge is slightly sticky as above mentioned. If the sponge is inclined to flake off, heat the instrument, dip in some light oil to prevent sticking and the piece may be pressed into position. To remove, heat a sharp pointed explorer and drive in the center of the mass. Cool with 100 water and the gold will come out in one piece. Coat the cavity surface of the filling with casting investment taking care not to 105

let any get on the surface in which the explorer is inserted. When the investment sets heat the instrument near the filling and it will easily remove without disturbing the gold.

5 After having prepared the sponge to fit the cavity as described the prepared sponge is placed on an asbestos mat, cavity side down, in an electrical or gasolene oven or in the flame of a blow torch. Heat the piece gradually to drive off the gum, since if hastened at first the pieces will blister. Place on top of the filling metal clippings of lower karat to the quantity which the 10 sponge will absorb without excess. A liquid surface when melted will indicate that the sponge is satisfied. The instant the pieces are seen to melt withdraw them for examination. As long as a rough surface is presented the sponge is still unsatisfied and more clippings are required.

15 In cases where walls of compound cavities and simple cavities are properly shaped, a matrix may not be necessary. However in cases where a matrix is thought to be 20 advantageous proceed as follows: The cavity is prepared in the same way as for any inlay filling. To conserve gold the cavity if too deep may be partly filled with cement 25 or other suitable material. The matrix may be made very satisfactorily of pure thin plate gold, for instance No. .002 SSWG. In case of large fillings a piece of paper is 30 trimmed to size for pattern and the gold plate cut to it. The gold plate is then placed over the cavity and pressed to place with a wet pellet of cotton. The gold is 35 then removed and annealed and pressed into place a second time, it making no difference if the bottom of the gold tears. 40 After thus preparing the matrix it is filled with sponge gold in the same manner as previously described in the case of a simple cavity, and the inlay prepared by melting 45 in additional pieces of metal, also as previously described. If the cavity is in an occlusal surface have the patient bite in the gold the same as if taking a wax impression of the cavity for a casting. In this 50 way an occlusion may be procured as correct as if a wax impression were made for a casting and with about an equal amount of trouble. In case of a compound cavity an ivory matrix should be used as just described, disengaging the clamp when the 55 bite is to be taken. When complete remove the entire piece for firing.

60 The fillings with matrices do not require investing, but after baking should have the surfaces to be cemented slightly roughened by rolling over with a small bur. The cementing process is the same as any other inlay process and need not be described here. Bridges and gold plates may be made 65 in a manner similar to fillings. Pure gold

matrices of thicker gold than for inlays are used. Since these pieces are of large size it is probable that they will need to be baked in the flame of a blow torch, since the average dental furnace is of too small a size. 70 To prevent warping the matrix must be pinned to the model. Pins may be made of platino iridium wire bent short and sharply at one end to act as a head. The pins should be distributed around the matrix as the case demands.

75 It will be obvious that while the method herein described was developed primarily for use in connection with dental work, it can be readily applied to the preparation 80 of articles for other purposes, such as the manufacture of articles of jewelry for personal wear, or gold and silver dishes and similar articles.

Having thus described my invention, 85 what I claim as new and desire to secure by Letters Patent is:

1. The method of making metal articles which consists in preparing a porous metal sponge of the shape desired, and fusing into 90 said sponge metal to fill the pores thereof and to enable it to retain its original shape under pressure.

2. The method of making metal articles which consists in preparing a metal sponge 95 and fusing into said sponge metal of the same character but of a lower melting point.

3. The method of making metallic sponge which consists in mixing metal particles or 100 fibers with a semiliquid binder and subjecting the resulting mass to the action of heat.

4. The method of preparing metal sponge which consists in mixing spongy metal with a semiliquid binder and subjecting the resulting mass to the action of heat. 105

5. The method of making a metallic sponge which consists in preparing a semiliquid binder by dissolving resin in cocoanut oil, adding said binder to spongy metal and subjecting the resulting mass to the 110 action of heat.

6. The method of making gold inlays which consists in mixing spongy gold with a semiliquid binder, subjecting the resulting mass to the action of heat to form a 115 plastic, adhesive metal sponge, molding the said metallic sponge to the shape of the cavity to be filled and fusing into said sponge gold of a lower melting point than the first mentioned gold. 120

7. The method of making gold sponge which consists in mixing spongy gold with a binder and heating the resulting mass to a temperature below red heat.

8. The method of making metallic sponge 125 which consists in preparing a binder by dissolving a wax-like material in a vegetable oil, and intimately mixing small pieces of metal with said binder.

9. The method of making metal articles 130

which consists in preparing a metal sponge and fusing into said sponge other material of a lower melting point.

10. The method of preparing gold sponge which consists in mixing sponge gold with a binder and heating the resulting mass to a temperature below red heat.

11. The method of making articles which consists in mixing small pieces of material with a destructible binder to form a sponge, forming the sponge into the shape desired, heating the sponge to drive off the binder and adding fused material to replace the binder in the pores of the sponge.

15. 12. The method of making articles which consists in mixing small pieces of material with a destructible binder to form a sponge, forming the sponge in the shape desired, heating the sponge to drive off the surplus binder, and adding fused metal to replace the binder in the pores of the sponge.

13. The method of making metallic

sponge which consists in preparing a binder by dissolving a wax-like material in an oil and intimately mixing small pieces of metal 25 with said binder.

14. The method of making plastic metallic sponge which consists in dissolving a solid component having the characteristic of being completely volatilizable by heat in 30 a liquid solvent to form an adhesive binder, mixing said binder with small pieces of metal, and heating the resulting mixture to a temperature below red heat to dispel the excess of solvent and to insure a complete 35 mixing of metal and binder.

In witness whereof, I hereunto subscribe my name this twenty-second day of July A. D. 1911.

FREDUS ALEXANDER THURSTON.

Witnesses:

AUGUSTUS S. DENNISON,  
O. M. WERMICH.